

June 5, 1923.

1,457,977

I. KITSEE

PRODUCING ARTIFICIAL SILK

Filed Oct. 25, 1921



## UNITED STATES PATENT OFFICE.

ISIDOR KITSEE, OF PHILADELPHIA, PENNSYLVANIA.

## PRODUCING ARTIFICIAL SILK.

Application filed October 25, 1921. Serial No. 510,246.

*To all whom it may concern:*

Be it known that I, ISIDOR KITSEE, citizen of the United States, residing at Philadelphia, in the county of Philadelphia and 5 State of Pennsylvania, have invented certain new and useful Improvements in Producing Artificial Silk, of which the following is a specification.

My invention relates to an improvement in 10 producing artificial silk and has more special reference to the production of artificial silk with the so-called cupro-ammonium process.

In application Serial No. 502,866 of Sept. 15 24, 1921, I have illustrated and described the means to generate the required gases at the point of using the same for the conversion of the fiber into required viscosity. In Letters Patent No. 1,390,995 of Sept. 20, 20 1921, I have described a process with the aid of which the dissolving action of the fiber is greatly exhilarated. In Letters Patent No. 1,389,517 of Aug. 30, 1921, I have illustrated and described means to produce 25 the thread out of the viscous mass in a greatly improved manner as is practiced today. The main object of this invention is to produce what I call a "working unit" with the aid of which the raw fiber may be converted into a finished thread, colored if desired, automatically without necessitating the removal of the fiber in the different stages of operation, from the device. In other words to produce a silk thread to be 30 used commercially without manual labor from the time that the raw fiber is placed in its compartment, till the finished thread is taken—colored if desired—from the spool on which it is wound, thus saving a great deal of labor and expense necessary with the 35 processes of today.

In the drawing which illustrates one form 40 my invention may take, Fig. 1 is a vertical sectional view partly in elevation, illustrating diagrammatically the different parts of the "unit" to be employed in accordance with this my invention. Fig. 2 is a section of the converting chamber of the "unit."

The "unit" consists here of the generating 45 chamber A, the converting chamber B, the storage tank C and the coagulating and spinning compartment D.

The generating chamber A comprises here 50 the casing 2 containing the liquid 3 and comprising the hoppers 4 and 5 for the ammonium salt and calcium oxide respectively and

provided each with a measuring device 6 and valve 7; it also comprises the agitator 8 adapted to be revolved through means 9. To the casing is attached the pipe 10 provided with the valve 11 and water gauge 12. It is also provided with a pressure and safety gauge 14 and the manhole 16. The operation of this part of the "unit" is clearly described in the application above mentioned.

The converting chamber B comprises here the casing 17 inclosing the agitators. These agitators comprise here the revolvable gears 20 fulcrumed each at 19 and provided each 55 with the wings 18. These agitators are revolved with the aid of the pinion 21 fulcrumed at 22. The motive power may be mechanical or electrical. In this casing, the required fiber and liquid is introduced 70 through manhole 23. The method of producing viscosity of the fiber is set forth in Letters Patent No. 1,390,995 above cited.

The coagulating and spinning compartment D comprises here the casing 38 provided here with the stationary receptacle 30 for the converted solution and the revolvable base 31 with its appended nipples or nozzles 32. The revolvable part 31 is operated through the gears 39, the shaft of 80 which may be revolved with the aid of mechanical or electrical means. The fibers issuing from the nozzles 32 are indicated by 33 and the thread spun from these fibers by 34. The compressing means for this thread are indicated by 35 and the spool on which the thread is wound is indicated by 36. 37 are the means to revolve this spool in conjunction with the means to revolve the base 31. The casing contains the coagulating 85 agent. The mode or method of operating this part of the device is clearly set forth in Letters Patent No. 1,389,517 aforesaid.

In the practical working of the device I have found, that it is necessary to insert 90 between the converting chamber and coagulating and spinning chamber a storage tank C so as to insure a continuous operation. This tank C is here indicated by 26. It is connected on the upper side through pipe 100 24 to be closed by 25 with the converting chamber B and on its lower side through pipe 27 provided with valve 28, with the interposition of a force pump 29 with the stationary receptacle 30 through 105 pipe 27.

The chamber A is connected to chamber

B through pipe 13 provided with safety and pressure gauge 14 and valve 15.

Generally speaking, the gases are generated in A and are conveyed into B, where-  
5 in the raw fiber is converted through the gases and friction on the casing 17 and wings 18 in the presence of moisture into desired viscosity. It is obvious that the casing should either consist or be lined with  
10 copper and so also should the wings consist or be lined with copper. The semi-fluid viscous mass may run or be drawn into the storage tank 26 and from there be conveyed into the stationary receptacle 30.  
15 The pump 29 should exert pressure enough, so as to force the semi-fluid out of the noz-  
zles or nipples in the form of fine streams to be coagulated in the coagulating bath. This coagulating agent may be colored with  
20 a suitable dye. This in broad outlines em-  
braces the continuous process of producing economically the desired thread out of the raw fiber.

In application above mentioned I have  
25 illustrated one means of producing the re-  
quired friction between the fiber and the copper. In this application these means vary in detail from the one above referred to, but the end-result will be similar in both  
30 cases, I have illustrated one converting chamber as to be connected to the generating chamber A, but it is obvious and does not need further illustration, that a num-  
ber of these converting chambers may be  
35 connected on one side with one generating chamber and on the other side with one storage tank, so also is it obvious that a series of coagulating and spinning compartments may connect with one and the same  
40 storage tank. I have illustrated the base 31 and the screw of the spool 36 as to be revolved together, but it is obvious that each of these devices may have separate actuating means. In some cases, this separation  
45 may even be preferred, but I do not deem it necessary to illustrate this modification.

Having now described my invention, what I claim as new and desire to secure by Letters Patents is:

50 1. In the production of artificial silk the method which consists in causing in one continuous operation automatically to be produced a desired thread comprising a series of filaments out of the raw fiber with-  
55 out necessitating the removal of the fiber

during the different stages of operation from the source of supply and without al-  
lowing the atmospheric air to contact with the products during the different stages of production.

2. In the production of artificial silk the method which consists in causing to be pro-  
duced the gaseous agent required for the conversion of the fiber and causing then the converted fiber to be spun into a desired 65 thread in one continuous operation with-  
out requiring manual manipulations during the different stages of operation and with-  
out allowing the atmospheric air to contact with the products during the different 70 stages of production.

3. The process of producing the convert-  
ing agent as well as the conversion of fiber and its formation into a thread through the operation of one working unit, continuously 75 and automatically and without allowing the atmospheric air to contact with the products during the different stages of production.

4. In the production of artificial silk the improvement which consists in converting 80 with the aid of nascent ammonia gas in conjunction with copper, cellulose fibers into a viscous mass, and coagulating and spinning said coagulated mass into required threads through the operation of devices 85 comprising one working unit and without allowing the atmospheric air to contact with the products during the different stages of production.

5. A device comprising a mechanical unit 90 adapted to produce artificial silk, said device comprising a chamber, generating the required solvent, a converting chamber for producing the required viscous mass connected to the first named chamber, a reser- 95 voir for the viscous mass connected to the converting chamber and a spinning device connected to said reservoir.

6. In a device of the class described a chamber for generating gases, a convert-  
ing chamber to convert a fiber into a viscous mass, a reservoir for said mass and a coagulating and spinning chamber for the converted cellulose and conveying means connecting the different chambers and reser- 100 voir to each other.

In testimony whereof I affix my signa-  
ture.

ISIDOR KITSEE.